

March 7, 1939.

P. L. MENAUL

2,149,617

METHOD AND APPARATUS FOR HANDLING ACIDIC SOLUTIONS

Filed Dec. 19, 1936

2 Sheets-Sheet 1



Fig. 1.



Fig. 2.



Fig. 3.

INVENTOR.  
Paul L. Menaul.

BY *Paul Babcock*  
ATTORNEY

March 7, 1939.

P. L. MENAUL

2,149,617

## METHOD AND APPARATUS FOR HANDLING ACIDIC SOLUTIONS

Filed Dec. 19, 1936.

2 Sheets-Sheet 2

Fig. 6.



Fig. 4.



Fig. 7.



Fig. 5.



INVENTOR.  
Paul L. Menaul.  
BY Earl Babcock  
ATTORNEY

## UNITED STATES PATENT OFFICE

2,149,617

METHOD AND APPARATUS FOR HANDLING  
ACIDIC SOLUTIONS

Paul L. Menaul, Duncan, Okla., assignor to Halliburton Oil Well Cementing Company, Duncan, Okla.

Application December 19, 1936, Serial No. 116,768

11 Claims. (Cl. 166—1)

This invention relates to method and apparatus for handling acidic solutions, and more particularly to electro-chemical means and method for protecting metals against corrosion caused by exposure of the metals to strong acids.

This application is in continuation in part of the copending application of Paul L. Menaul, Serial No. 77,945, filed May 5, 1936, for "Method and apparatus for handling acidic solutions."

10 Strong solutions of hydrochloric acid and other acids attack various metals, and the present invention is intended to protect metals, particularly iron, from the corrosive action of such acids.

It is known to the art to protect metals from 15 weak acids by electrical means, but the methods heretofore employed for this purpose are generally ineffective in protecting metals from strong acids.

It is one object of the present invention to protect iron and other metals from strong acids by 20 electro-chemical means and methods which will effectively pacify them with respect to the acid without impairing the normal properties of the acid to any material extent.

25 A further object of the invention is to provide means and methods of acid-treating oil wells or the like whereby corrosion of metallic equipment, such as casing or tubing, in contact with the acid or acid solution is retarded.

30 Other objects and advantages reside in certain novel features of the arrangement and method, as will be apparent from the following description taken in connection with the accompanying drawings, in which:

35 Fig. 1 is a diagram illustrating an iron and a lead electrode in a beaker of hydrochloric acid, the arrangement illustrating some principles of the invention.

Fig. 2 is a diagram similar to Fig. 1, but illustrating a slightly different arrangement.

40 Fig. 3 is a diagrammatic illustration, in vertical cross-sectional view, of an oil well and illustrating one embodiment of the invention applied thereto to protect the metal therein.

45 Fig. 4 is a diagrammatic illustration of a modified form of the invention as applied to an oil well.

Fig. 5 is a vertical cross-sectional view of a container for acid constructed in accordance with the invention.

50 Fig. 6 is a diagrammatic illustration of the upper portion of an oil well, together with a tank constructed in accordance with the present invention for supplying acid to the well and a pump for forcing the acid from the tank into the well;

55 and

Fig. 7 is a diagrammatic illustration of a tank and well similar to that of Fig. 6, but illustrating a modified arrangement.

In describing the invention, some underlying principles will first be explained and this will be 5 followed by a disclosure of some adaptations of these principles to oil well equipment to which they are particularly applicable.

When two electrodes of different metals are immersed in an electrolyte, a difference in electrical potential is created between them and current tends to flow from one to the other through 10 the electrolyte.

The difference in potential and the direction of flow of current depends upon the nature of 15 the electrodes selected and possibly in some cases on the nature and condition of the electrolyte.

Metals may be arranged in what is called a voltaic series or electro-chemical series, the position of any given metal in the series being determined by the direction of flow of current through the electrolyte from that metal to any other in the series, when terminals on the electrodes are connected by an electrical conductor exterior to the electrolyte.

The current flows through the electrolyte from what is herein termed the more electro-positive plate or element to the other, and then back to the electro-positive plate or element through the 20 external conductor.

In a galvanic cell like that shown in Fig. 1, having iron as one electrode and commercial sheet lead as the other electrode, with hydrochloric acid as the electrolyte, the lead electrode is electro-positive with respect to the iron electrode.

The iron becomes the positive pole of the cell and externally the current flows from the terminal of the iron electrode to the terminal of the lead electrode. The voltage causing this current 30 is very low, being only about 100 millivolts.

This voltage is in the proper direction to tend to protect the iron against corrosion, since the current is flowing from the acid to the iron, but because this force is very small, it is ineffective 40 for this purpose and, for a time, corrosion of the iron takes place.

However, this corrosion does not continue. The 45 corrosion of the iron by the hydrochloric acid soon diminishes to a negligible amount. The explanation for this phenomenon must be found elsewhere than on the basis of a mere difference in electrical potential, it being known that such small voltages are not capable of producing the desired result.

25

30

35

40

45

50

55

Now, it is known that lead may be deposited on iron by causing an electric current to pass through hydrochloric acid in which the lead has been dissolved, and the most obvious explanation for the above described phenomenon is that some lead has gone into solution in the acid and become deposited on the iron, thus forming a protective coating or lead plate on the iron.

An examination of the iron electrode after a time shows this to be a fact. There is a visible but immeasurably small deposit of lead thereon. But if this electrode is now placed back into the acid with the lead electrode removed, after a time corrosion starts up again and once it starts it continues at a more rapid pace than ever, both the lead and the iron going into solution in the acid. This minute deposition of lead on the iron may have something to do with the prevention of corrosion, but it seems clear that other than electroplating factors are involved and that the extremely small amount of lead deposited is ineffective per se, to obtain the desired result.

It is thus seen that in the cell mentioned, the voltage or the difference in potential is insufficient to obtain protection and that the extremely small deposition of lead on the iron is insufficient to form a protective insulating coating.

The results obtained, therefore, must be due to the combination of difference in potential and the electroplating of lead on the iron. This leads to consideration of what is called "hydrogen over-voltages", a discussion of which is believed to be necessary in order to understand not only the basic underlying principles of the behavior of iron and lead in the example given above but also the broader adaptations of the invention to metals and electrolytes other than those mentioned herein.

It is known that when an electrode is placed in an acid, and current is passed from the acid to the electrode, hydrogen is disassociated from the acid and passes off as bubbles. There is little or no bubbling off of the hydrogen however until the certain critical voltage between the acid and the metal is reached. This critical voltage is called the "decomposition voltage" of the electrolyte.

It is further known that the "decomposition voltage" varies, depending on the nature of the electrodes. The difference between the actual potential at which there is visible evolution of hydrogen gas with a certain metal as electrode and the potential at which decomposition starts in the same solution with a hydrogen electrode, is called the "hydrogen over-voltage" of that metal.

Now, lead has a much greater "hydrogen over-voltage" than iron in hydrochloric acid, and it is believed that the very slight deposition of lead on the iron in the example given above, while ineffective to isolate the iron completely from the acid, is effective to increase the "hydrogen over-voltage" of the iron electrode. The iron cannot go into the solution in the acid unless hydrogen molecules are liberated, and the abnormal hydrogen over-voltage prevailing on the iron electrode, due to the lead thereon, coupled with the small difference in potential resulting from galvanic action, prevents this taking place. This is believed to be the theory underlying the peculiar behavior of iron and lead in the example given and it is thought that the same principles may be applied to other metals.

If desired, the normal difference in potential between the plates of the cell of Fig. 1 may be altered (preferably increased) by an external

battery. Such an arrangement is shown in Fig. 2. The operation of this arrangement is the same as that in Fig. 1 except that the voltage between the plates may be altered to best suit the conditions.

As mentioned above, commercial sheet lead was used as the anode in the galvanic cells described above to illustrate the above principles.

Commercial sheet lead was selected because it appears that with iron and with hydrochloric acid, the galvanic cell thus constructed has just the right voltage to give the desired protection without any considerable amount of the lead going into the solution.

One peculiarity in the behavior of iron which has been used for some time as an electrode in a cell like that described is that it has become temporarily pacified. After the thin film of lead has been deposited thereon for some time, the lead electrode may be removed and so long as the iron electrode is not disturbed, the acid will remain inactive with respect to it for quite some time. This is probably due to the adsorption of hydrogen by the lead film from the acid.

On the accompanying drawings, several adaptations of the above principles to oil well equipment are shown.

Referring to Figs. 3 to 7 of the drawings in detail, and first to the arrangement of Fig. 3, the well hole indicated at 1 contains a casing indicated at 2 which terminates at the top of an oil-bearing strata 3. In accordance with customary practice, the casing is shown cemented in the hole, the cement being indicated at 4. Extending downwardly through the casing is a well pipe 5 which extends beyond the casing into the well bore puncturing the formation 3. The well pipe 5 may carry a packer 6 blocking the upward passage of fluid through the annular space between the well pipe 5 and the casing 2. The casing head and other devices commonly found at the top of a well hole are not shown.

In acid treating the formation 3 for the purpose of increasing its porosity or removing obstructing matter which restricts flow of oil into the well hole, an acidified solution such as, for example, a 15% hydrochloric acid solution, is pumped downwardly through the pipe 5 into the formation. In practice, the solution is pumped into the formation for an appreciable period of time of, say, from several hours to several days. Since the acid is in contact with the casing or tubing or both while being placed in the well, it may corrode the same. In accordance with this invention, however, a metallic member such as a cable or wire is let down through the pipe 5, such wire being indicated at 7.

The wire or member 7 is preferably of a metal which is electro-positive to the metal of the well pipe 5. For example, since most well pipes are of iron, the wire 7 may be formed of commercial lead, a lead alloy, or it may be lead sheathed cable which externally of the electrolyte has been found to have a more negative potential than iron in hydrochloric acid. The lower end of the wire may be provided with a large weight, such as the lead weight 8. A metallic electrical conductor, such as a copper wire, is then attached to the metallic member or wire 7 and to the well tubing or pipe 5 at or near the top of the tubing. Such electrical conductor is indicated at 9.

It will be noted that the wire 7 is immersed

in the acid solution indicated at 10, such acid solution contacting not only the wire 7 but also the interior of the well pipe 5. When the metal of the wire 7 has a negative external potential 5 to iron (which forms the major element of the well pipe 5), then in effect a very inefficient battery is formed by the elements described and the electrodes become polarized, which decreases and in effect prevents the acid from corroding 10 the pipe 5.

As explained above in connection with Fig. 2, in certain cases it has been found desirable to apply an additional potential to plates of the cell, such potential being in the same direction 15 or polarity as the electromotive force which is attained by the use of the pipe, electrode and acidic solution alone. For this reason the positive pole of a battery or applied electromotive force may be connected to the lead electrode in 20 the well, which is in the acid solution, and the negative pole of the battery or applied potential may be connected to the iron casing or the metal which is to be protected. As indicated in Fig. 4, for example, the external circuit 9 may 25 include a battery or other source of electrical energy. The precise voltage or amperage of this source need not necessarily be fixed or critical. It has been found, for example, that by using 1 or 2 cells of a storage battery furnishing approximately 2 or 4 volts is sufficient to give the 30 desired polarization and obviate corrosion.

As a matter of fact, when a sufficiently large potential is applied in the external circuit 9, such a potential being superimposed on the 35 E. M. F. normally obtained by the pipe, electrode and acidic solution, an electrolytic action may take place whereby migration of considerable lead from the electrode 7 to the interior walls of the pipe 5 is attained. This electro-deposition of lead upon the interior surfaces is 40 usually exceedingly minute but does form a protective coating thereon, but excessive external voltage should not be applied. At about 4½ volts, for example, a spongy lead deposit may be formed on the interior of the tubing, which spongy lead 45 does not adhere with any great tenacity and often falls off when it is disturbed.

The electrode cable 7 may be introduced into the well either prior to the introduction of acid 50 solution or immediately thereafter. The cable should be of sufficient weight and of a sufficiently large size so that in the event any electrolytic action does take place, it does not completely disintegrate before the termination of the acid treatment.

The method of this invention may also be applied to the treatment of tanks or other containers in which acid is stored or shipped. A suitable plate of metal having a more negative external potential than iron in the acid solution, 55 for example, lead, is suspended in the acid and connected to the iron or steel tank, either with or without the medium of a battery or other source of low voltage direct current. As shown in Fig. 5, for example, the iron tank 12 may have a lead plate 13 in electrical contact with the bottom of the container. Such contact may be attained either by riveting or burning the lead into place. It is to be remembered that the lead 60 plate or lining should not cover the entire interior surface of the tank but only a part thereof so that the acid contained therein may contact with both the lead and the sheet iron. Desired polarization of the interior of the tank is thus 65 attained.

A particularly effective way of protecting both the tank used in conveying the acid to the well and also the casing, tubing or other metal parts of the well is shown in Fig. 6. This was disclosed to some extent in claim 8 of the copending application referred to above. 5

In Fig. 6 an iron tank for conveying the acid is illustrated at 14. The tank may be mounted on a truck or trailer and obviously may be of any desired shape. 10

A lead plate 15 is burned or otherwise secured to the tank 14 so as to provide at least one point where it forms a good electrical connection therewith. 15

The galvanic cell set up by the lead plate and 15 the iron tank when strong hydrochloric acid is placed therein effectively protects the tank, as explained above in connection with Fig. 3.

Upon arriving at the oil well into which the acid is to be pumped, an electrical conductor or 20 cable 16 is connected between the tank 14 and the casing or tubing 17 of the well. The conductor 16 may be permanently welded to the tank as shown at 18 and may be clamped to the casing as shown at 19. Any other way of effecting good 25 electrical contact will serve the purpose.

If now a pump, such as that diagrammatically shown at 20, is operated to cause the acid in the tank to flow through the acid conduits 21 and 22 in the well, an electric circuit will be set up and 30 current will flow from the acid in the well to the casing 17, the electrical conductor 16, the tank 14 and the lead plate 15 back to the acid.

The effect is the same as though the casing 17 35 became part of the tank 14, and corrosion of the casing 17 will not take place, even though it is several thousand feet in length.

It is remarkable to note that casing many thousand feet from the lead plate 15 is pacified. The explanation for this may be that both the acid and 40 the casing are good conductors of electricity, but it is believed that an additional factor is involved, namely, that as soon as one part of the casing becomes pacified, the resistance of that part immediately goes up. This is in harmony 45 with the theory that a film of lead or hydrogen or both is formed on the iron since such a film would present a higher hydrogen over-voltage and likewise cause a high resistance to develop. This would increase the current density adjacent other parts of the well. A film would tend to form wherever it did not already exist and once formed would tend to cause the current to flow from the acid to the casing somewhere else which in turn would tend to cause the formation of a film there, 50 and so on, every part of the casing being protected as soon as that part is contacted by the acid. 55

It may be desirable in some instances to supplement the voltage generated by the galvanic action in the tank of Fig. 6 by an auxiliary source of direct current potential and an arrangement for accomplishing this is shown in Fig. 7. 60

The system in Fig. 7 is the same as that in Fig. 6, except that a storage battery or the like 65 has been connected into the conductor 16, as shown at 23. This battery must be so connected as to cause current to flow from the casing 17 to the tank 14, since this is the direction of flow caused by the galvanic action in the tank. 70

Whether an auxiliary source of potential is employed or not, the conductor 16 may be connected to the tank almost anywhere, but it could equally well be connected to the plate 15 directly. The electrical resistance of the tank being low, 75

the point of connection of the conductor 16 there-to does not make much difference.

Another peculiarity of the invention is that it does not make much difference what kind of material is used for the acid conduits 21 and 22. If these conduits are of iron they are connected to the tank through the casing 17 and conductor 16 and are readily pacified. If rubber or canvas hose is used it makes no difference because a path for the flow of current is provided by the acid itself from the acid in the tank to the acid in the well.

When an auxiliary source of potential is used, as shown at 23, in Fig. 7, the voltage must not be too high, preferably not over 4 to 6 volts, or considerable lead will go into the solution and be deposited on the iron. This does not do any harm, other than being wasteful, but neither does it do much good in protecting the casing or tank. It would be practically impossible to lead-coat the entire casing and the protection can be just about as effective with only a trace of lead being in the solution.

On the other hand, unless some lead does go into solution, what protection there is is wholly insufficient. A high direct current potential connected as illustrated in Fig. 7, in the absence of any lead in the tank 14, would not accomplish the purpose of the present invention.

In the following claims, where "hydrochloric acid" is recited, various solution concentrations are intended to be included; where "iron" is recited, various alloys of iron or steel are intended to be included; and where "lead" is recited, various alloys in which lead is the principle ingredient are intended to be included.

It will thus be clear that although only a few embodiments of the invention are shown and described herein, the principles are of broad application and that many changes may be made, both in the structure and method, without departing from the spirit of the invention or the scope of the annexed claims.

I claim:

1. A method of acid treating wells which includes introducing hydrochloric acid into the well hole and into contact with the earth structure to be treated through and in contact with an iron well pipe, introducing a lead electrode into the well pipe and into contact with the acid and electrically connecting said pipe and electrode.

2. A method of acid treating wells which includes introducing hydrochloric acid into the well bore and into the earth structure to be treated through an iron well pipe, introducing a lead electrode into the well pipe and into contact with the acid, and applying a direct current potential to the electrode and pipe, the negative pole of the applied source of current being connected to the well pipe and the positive pole being connected to the aforesaid electrode in acidic solution.

3. A method of acid treating wells which includes introducing hydrochloric acid from an iron tank into a well bore and into contact with the earth structure to be treated through an iron well pipe; electrically connecting a lead electrode to said tank, the electrode being in contact with the acid but not covering all of the tank in contact with the acid, and electrically connecting the tank to the well pipe.

4. A method of protecting from corrosion an

iron vessel containing hydrochloric acid in contact with said vessel which includes electrically connecting a lead electrode to the vessel, said electrode being in contact with the acid therein.

5. The method of protecting from corrosion, a body of iron exposed to and in contact with hydrochloric acid which includes placing a lead electrode in the acid and electrically connecting the electrode to the body of iron.

6. Apparatus for acidizing an oil well and for protecting the iron equipment thereof during the placing of hydrochloric acid therein which includes, in combination with the iron equipment of the well, an iron tank adapted to hold the acid, an electrode of lead in the tank and so positioned as to contact the acid, means for electrically connecting the tank to the iron equipment, and conduit means for conveying the acid from the tank into the well, said conduit means being so arranged as to provide an electrical connection from the acid in the tank to the acid in the well through the acid in said conduit means when the acid is flowing therethrough.

7. Apparatus for acidizing oil wells with hydrochloric acid which includes an iron pipe in the well, an iron tank adapted to contain the acid to be supplied to the well, said tank having a plate of lead electrically connected thereto in contact with the acid therein, a pump for pumping the acid from the tank into the well, acid conduits connecting the tank to the pump and the pump to the well, and means for electrically connecting the tank to the pipe in the well.

8. The method of protecting iron in contact with hydrochloric acid from corrosion due to that contact which includes dissolving a trace of lead in the acid, electrically depositing a film of the lead so dissolved on the iron and impressing a low voltage of direct current between the acid and the iron to maintain the film on the iron.

9. The method of protecting iron in contact with hydrochloric acid from corrosion due to that contact which includes placing a body of lead in the acid to cause a trace of the lead to be dissolved in the acid, electrically depositing some of the lead so dissolved on the iron to form a protective coating thereon and impressing a low voltage of direct current between the acid and the iron to maintain said coating.

10. The method of protecting iron in contact with hydrochloric acid from corrosion due to that contact which includes placing a body of lead in the acid to cause a trace of the lead to be dissolved in the acid, electrically depositing some of the lead so dissolved on the iron to form a protective coating thereon and impressing a low voltage of direct current between the acid and the iron to maintain said coating, said voltage being maintained by causing galvanic action in the acid by electrically connecting the lead to the iron.

11. The method of increasing the output of a petroleum well by treating a petroleum bearing formation with acid, while protecting iron bodies in the well which includes the steps of connecting a conduit to the well and to a tank containing the acid, causing the acid to flow from the tank into the well and electrically pacifying the acid with respect to the iron bodies in the well by placing a lead electrode in the acid in the tank and electrically connecting the electrode to the tank and to the iron bodies.

PAUL L. MENAUL.